

# United States Patent [19]

Jaeckel et al.

[11] Patent Number: 4,883,495

[45] Date of Patent: Nov. 28, 1989

[54] AMINO-CONTAINING ALKENYLSUCCINIC ESTERS

[75] Inventors: Lothar Jaeckel, Flörsheim am Main; Rolf Kleber, Neu-Isenburg; Bernhard Mees, Eppstein, all of Fed. Rep. of Germany

[73] Assignee: Hoechst Aktiengesellschaft, Frankfurt am Main, Fed. Rep. of Germany

[21] Appl. No.: 247,277

[22] Filed: Sep. 21, 1988

## [30] Foreign Application Priority Data

Sep. 25, 1987 [DE] Fed. Rep. of Germany ..... 3732340

[51] Int. Cl.<sup>4</sup> ..... D06M 9/00; C07C 69/593

[52] U.S. Cl. ..... 8/115.6; 8/115.51; 560/196; 560/204

[58] Field of Search ..... 560/196; 8/115.51, 115.6

## [56] References Cited

### U.S. PATENT DOCUMENTS

4,185,485 1/1980 Shick et al. ..... 560/196 X  
4,435,297 3/1984 Forsberg ..... 560/196 X  
4,734,523 3/1988 Hofinger et al. ..... 560/196

Primary Examiner—Werren B. Lone  
Assistant Examiner—Vera C. Clarke

## [57] ABSTRACT

Amino-containing alkenylsuccinic esters of the formulae



and



where R denotes linear or branched C<sub>1</sub>-C<sub>20</sub>-alkyl, R<sub>1</sub> denotes hydroxy-C<sub>2</sub>-C<sub>6</sub>-alkyl or C<sub>1</sub>-C<sub>4</sub>-alkyl, R<sub>2</sub> denotes methyl or ethyl, R<sub>3</sub> denotes C<sub>6</sub>-C<sub>20</sub>-alkyl, preferably C<sub>12</sub>-C<sub>18</sub>-alkyl, or C<sub>6</sub>-C<sub>20</sub>-alkenyl, preferably C<sub>12</sub>-C<sub>18</sub>-alkenyl, A denotes —C<sub>2</sub>H<sub>4</sub>— or C<sub>3</sub>H<sub>7</sub>— and n denotes a number from 1 to 10, preferably from 3 to 8, the preparation thereof and the use thereof as thermostable lubricants in spin finishes.

9 Claims, No Drawings



The Examples which follow are intended to illustrate the invention without limiting it.

## EXAMPLE 1

In a 250 ml vessel equipped with stirrer, internal thermometer and short path distillation attachment, 53.38 parts by weight of n-dodeceny succinic anhydride are melted at about 50° C., and 18 parts by weight of N,N-dimethyl ethanolamine are added dropwise with stirring under nitrogen at 50° to 55° C. in the course of 10 30 minutes. The thick emulsion is stirred at 50° C. for 4.5 hours until anhydride is no longer detectable by thin layer chromatography. The mixture is cooled down to 30° C., and 86.3 parts by weight of a coconut alcohol ethoxylate (incorporating 5 ethylene oxide units), 1.2 15 parts by weight of ultrapure boric acid and 1.7 parts by weight of hypophosphorous acid (50% strength) are added. This is followed by 4 hours of stirring at 150°-155° C. under nitrogen, during which a total of 4 ml of water are distilled off. This is followed by distillation under reduced pressure at a temperature between 130° to 155° C. for 3 hours to remove in addition 8 parts by weight of the starting compound, leaving 146 parts by weight of a pale brown, pourable compound having a pH (1% in water) of 6 to 7. 20 25

## EXAMPLE 2

Example 1 is repeated, except that n-dodeceny succinic anhydride is replaced by 50 g of i-nonenylsuccinic anhydride. About 45 g of a pale brown liquid having a 30 pH of 7 are obtained.

## EXAMPLE 3

In a 500 ml vessel equipped with stirrer, internal thermometer and short path distillation attachment, 70 parts by weight of n-octadecenylsuccinic anhydride are dissolved in 150 parts by volume of tetralin, and 21.6 35 parts by weight of N,N-diethyl ethanolamine are added dropwise with stirring under nitrogen at 35° C. in the course of 30 minutes. The mixture is left to react at 50° 40 C. for 4 hours and then cooled down to room temperature, and 107 parts by weight of stearyl alcohol with 6 moles of ethylene oxide and 3 parts by weight of p-toluenesulfonic acid are added. About 4 ml of water are distilled off at 160° to 180° C. in the course of 2 hours, 45 and then the tetralin is distilled off at 160° C. in an aspirator vacuum and recovered. About 190 parts by weight are obtained of a pale brown, viscous oil having a pH of 7. 50

## EXAMPLE 4

Example 2 is repeated, except that the 21.6 parts by weight of N,N-diethyl ethanolamine are replaced by 25 parts by weight of N,N-dimethylbutanolamine. About 193 parts by weight are obtained of a pale brown, viscous oil having a pH of 7. 55

The compounds obtained according to Examples 1 to 4 have the following structures:



-continued



## EXAMPLE 5

Heating test: 1 g samples of the following substances are weighed out into a thin aluminum dish which is heated at 220° C. for 24 hours and the losses determined:

- (a) mineral oil (viscosity at 20° C. : 300 mPas)
  - (b) pentaerythritol tetradecylate
  - (c) product according to Example 1
  - (d) product according to Example 2
  - (e) product according to Example 3
  - (f) product according to Example 4
- a+b: comparisons  
c-f: according to the invention

|     | Loss at<br>220° C./24 h | Residue        | Solubility of residue<br>in cold water |
|-----|-------------------------|----------------|----------------------------------------|
| (a) | 50%                     | black, solid   | insoluble                              |
| (b) | 60%                     | black, solid   | insoluble                              |
| (c) | 33%                     | yellow, greasy | emulsible                              |
| (d) | 40%                     | yellow, greasy | emulsible                              |
| (e) | 35%                     | yellow, greasy | emulsible                              |
| (f) | 30%                     | yellow, greasy | emulsible                              |

## EXAMPLE 6

## Friction values on PES

| Product | Pure oil |           | 5 g/l  |           |
|---------|----------|-----------|--------|-----------|
|         | static   | dynamic   | static | dynamic   |
| a       | 8.4      | 0.44-0.48 | 8.2    | 0.49-0.50 |
| b       | 8.5      | 0.48-0.59 | 8.3    | 0.49-0.55 |
| c       | 8.9      | 0.42-0.47 | 8.0    | 0.43-0.47 |
| d       | 8.3      | 0.44-0.48 | 8.1    | 0.44-0.49 |
| e       | 8.2      | 0.41-0.46 | 8.0    | 0.40-0.45 |
| f       | 8.2      | 0.43-0.49 | 8.1    | 0.41-0.46 |

a + b comparisons as per Example 5

c - f Examples 1 to 4 according to the invention

65 These values were determined by the method specified in German Offenlegungsschrift 2,355,675, specifically at measuring speeds of 25 m/min (first value) and 100 m/min (second value).

6

We claim:

### 1. A compound of the formulae



01



where R denotes linear or branched C<sub>1</sub>-C<sub>20</sub>-alkyl, R<sub>1</sub> denotes hydroxy-C<sub>2</sub>-C<sub>6</sub>-alkyl or C<sub>1</sub>-C<sub>4</sub>-alkyl, R<sub>2</sub> denotes methyl or ethyl, R<sub>3</sub> denotes C<sub>6</sub>-C<sub>20</sub>-alkyl, or C<sub>6</sub>-C<sub>20</sub>-alkenyl, A denotes —C<sub>2</sub>H<sub>4</sub>— or —C<sub>3</sub>H<sub>7</sub>— and n denotes a number from 1 to 10.

2. A process for preparing a compound as claimed in claim 1, which comprises reacting an alkenylsuccinic acid of the formula

1 30

40

45

50

55

60

65



or the anhydride thereof first with 1 mole of an amine of the formula



and then with 1 mole of an alkoxylated alcohol of the formula

$$\text{R}_3(\text{OA})_n-\text{OH}$$

where  $R$ ,  $R_1$ ,  $R_2$ ,  $R_3$ ,  $A$  and  $n$  are as defined in claim 1.

**3. A compound as claimed in claim 1, wherein:**

R denotes linear or branched C<sub>5</sub>-C<sub>15</sub> alkyl;

$R_3$  denotes C<sub>12</sub>-C<sub>18</sub>-alkyl or C<sub>12</sub>

25 n denotes a number from 3 to 8.  
4. A compound as claimed in claim 1, wherein R denotes linear or branched C<sub>5</sub>-C<sub>15</sub> alkyl.

5. A compound as claimed in claim 1, wherein  $R_3$  denotes  $C_{10}-C_{15}$  alkyl.

30 6. A compound as claimed in claim 1, wherein  $R_3$

7. A compound as claimed in claim 1, wherein n

35 8. A compound as claimed in claim 5, wherein n denotes a number from 3 to 8.

denotes a number from 3 to 8.

9. A spin-finish composition containing an effective amount of a compound of claim 1 and at least one additional spin-finish component.

\* \* \* \*

40